# NEW EUROPEAN PATENT SPECIFICATION

(11) **EP 1 349 914 B2**
(45) Date of publication and mention of the opposition decision: **04.09.2013**
(45) Mention of the grant of the patent: 16.12.2009
(21) Application number: 01272727.7
(22) Date of filing: 24.12.2001
(51) Int. Cl.: C11D 17/06, C11D 17/00, C11D 3/12

(54) **A PROCESS FOR THE PRODUCTION OF CLEANING AGENTS**
VERFAHREN ZUR HERSTELLUNG VON REINIGUNGSMITTELN
METHODE DE PRODUCTION DE PRODUITS DE NETTOYAGE

(30) Priority: 08.01.2001 GB 0100412
(43) Date of publication of application: 08.10.2003
(73) Proprietor: Reckitt Benckiser N.V., 2132 WT Hoofddorp (NL)
(72) Inventor: FRANZOLIN, Giorgio, I-30035 Mirano (IT); CORDELLINA, Antonio, I-35031 Abano Terme (IT); ROSA-FAUZZA, Luca, I-33100 Udine (IT)
(74) Representative: Brown, Andrew Stephen
(86) International application number: PCT/GB2001/005769
(87) International publication number: WO 2002/053697

(56) References cited:
- EP-A1- 0 512 552
- WO-A-01/34751
- WO-A1-91//02047
- WO-A1-95//29219
- WO-A2-91//15567
- DE-A- 19 948 671
- DE-A1- 3 926 253
- DE-A1- 4 034 131
- DE-A1- 4 125 330
- DE-A1- 19 808 757
- US-A- 5 376 288
- US-A- 5 382 377
- 'Sokalan® CP Marken' TECHNISCHE INFORMATION September 1998, pages 1 - 6

## Description

This invention relates to a method of making a solid laundry cleaning agent, in particular a laundry cleaning agent in pressed block form (hereinafter "laundry tablet"), but is also applicable to particulate laundry cleaning agents (hereinafter "washing powder"). Although discussion of the invention will focus on laundry tablets, washing powders are also of interest and share many of the advantages of the invention, that apply to laundry tablets.

A known laundry tablet comprises about 10% of a sodium (linear C₈₋₁₅ alkyl) benzene sulfonate, about 6 wt% of zeolite, about 12% of sodium carbonate, about 15% of sodium citrate dihydrate, about 20% of an amorphous silicate, present as a builder, about 10% of a cellulosic disintegrant and about 27% of additional ingredients (weight/tablet weight). Such a tablet is formed by simple dry mixing of a typical tower base powder with all the other ingredients, followed by tabletting the mixture in a standard tabletting machine, such as a Korsch rotating press.

This procedure and product is satisfactory but suffer from certain limitations. In particular, it would be advantageous to be able to incorporate a higher proportion of zeolite. However, higher proportions of zeolite in powder form would be expected to lead to unacceptably long disintegration times. It would also be advantageous to use a lower proportion of the disintegrant, which is an expensive component and one which is without benefit in terms of cleaning action. However, even small reductions would be expected to lead to unacceptably long disintegration times, especially with increasing zeolite proportion. Further, it would be advantageous to use a lower proportion of - or no - amorphous silicate, which is also expensive. Still further, it would be advantageous to offer smaller tablets with the same cleaning power. It would be desirable therefore to be able to make tablets of higher density provided that the disintegration time was still acceptably short. This is not an easy matter. Simply applying a higher compression force during tabletting achieves a higher density but at the expense of disintegration time, which may soon become unacceptable.

One possible approach was to consider using extruded particles which would then be mixed with further ingredients and pressed to form tablets. This approach is the subject of a number of patent applications of the company Henkel, of which we may mention EP-B-486592, (& US 5 382 377), by way of example. In EP-B-486592 there is described a process for the production of compacted granules for use in detergents. A homogenous premix, to which a plasticizer and/or lubricant is added, is extruded through perforated dyes under high pressure to form strands which are cut into pieces. There is preferably an unbound water content in the premix, preferably up to 12% by weight, more preferably up to 10% by weight and most preferably in the range from about 4 to 8% by weight. The premix may be of a tower powder. Zeolite is mentioned as a possible drying powder, to prevent the granules from sticking together, and as a possible premix component, albeit not in very high amounts.

When we attempted in our experimental work to evaluate this extrusion process using the types of laundry agents of interest to us, with a high proportion of zeolite, we did not find it to be of any potential use. The materials we wished to form into granules seemed insufficiently plastic to extrude well; indeed our extruder was damaged by the attempt.

We have now determined that, to our surprise, pelletisation - as distinct from extrusion - can be used as a key step in the manufacture of advantageous laundry tablets. Those laundry tablets can achieve the aims noted above - thus, they can be of high density; be small tablets; have high zeolite content; have low disintegrant content; fast disintegration; and have a low or no amorphous silicate content. Aside from advantageous laundry tablets the present invention offers the prospect of advantageous washing powders, with high bulk density, high zeolite content and low or no amorphous silicate content.

In accordance with a first aspect of the present invention there is provided a method of making a solid laundry cleaning agent, comprising the steps of pelletising a flowable tower spray powder and a flowable zeolitic powder in a pellet mill to form a premix comprising pellets with a zeolite content of at least 30% (weight of zeolite/weight of pellets); and mixing (hereinafter also called post-mixing) the pellets with the other ingredient(s) of the solid laundry cleaning agent, wherein the zeolitic powder is a zeolite admixed with up to 10% of a processing aid (weight of processing aid/weight of zeolitic powder including processing aid), the processing aid being selected from a nonionic surfactant, an acrylic polymer or copolymer; starch or a derivative thereof; gelatin; polyvinyl alcohol; soap; and water

Preferably the tower spray powder is made up of the following constituents (weight/weight of tower spray powder):
20-60% anionic surfactant; 0-15% processing aid; 0-25% further zeolite; 12-45% inorganic alkali metal, preferably sodium, salt; and. 0-20% additional constituent(s).

More preferably, the tower spray powder comprises 30-50% of one or more anionic surfactant.

Preferred anionic surfactants for the tower spray powder include (but are not limited to) alkali metal salts, ammonium salts, amine salts, aminoalcohol salts or magnesium salts of one or more of the following compounds: alkylsulphonates, alkylamide sulphonates, alkylarylsulphonates, olefinsulphonates, alkylamide sulphonates, alkyl sulfosuccinates, alkyl ether sulfosuccinates, alkylamide sulfosuccinates, alkyl sulfosuccinamate, alkyl sulfoacetates, acyl sarconsinates, acyl isothionates and N-acyl taurates. Generally, the alkyl or acyl group in these various compounds comprises a carbon chain containing 8 to 22, preferably, 12 to 20, carbon atoms.

Other anionic surfactants which may be used include salts (having cations as described above) of fatty acids, individually or as mixtures, including salts of oleic and stearic acids, and of acids of palm kernel oil, coconut oil and tallow; and lactylates whose acyl group contains 8 to 20 carbon atoms. Especially useful are solid soaps, and preferably solid alkali metal salts of C₁₆₋₁₈ saturated fatty acids, especially of tallow fatty acids, as these are useful also as processing aids.

An especially preferred anionic surfactant for use in the present invention is an alkali metal, preferably sodium, salt of a (C₈₋₁₅ - preferably C₉₋₁₃ linear alkyl)benzene sulphonic acid (hereinafter 8-15 LAS and 9-13 LAS).

Preferably an alkali metal salt of an alkylbenzene sulphonic acid (for example an LAS) is present in the pellets, preferably wholly derived from the tower spray powder.

Preferably an alkali metal salt of an alkylbenzene sulphonic acid (for example an LAS) is not present in the zeolitic powder which is to be pelletized. Preferably no anionic surfactant is present in the zeolitic powder which is to be pelletized.

Preferably an alkali metal salt of an alkylbenzene sulphonic acid (for example an LAS) is not present in the post-mixed ingredients to be mixed with the pellets.

Preferably the pellets do not contain any anionic sulphate surfactant.

Preferably the post-mixed ingredients include an anionic sulphate surfactant, suitably providing 2-10%, preferably 3-7%, of the final cleaning agent (weight/weight). Suitable anionic sulphate surfactants may include alkyl sulphates, alkyl ether sulphates, alkylamidoether sulphates, alkylaryl polyether sulphates, monoglyceride sulphates. Especially preferred are alcohol sulphates. Generally an alkyl group in these sulphate compounds is a C₈₋₂₂, preferably C₁₂₋₂₀, alkyl group.

The processing aid improves the efficiency of a later pelletisation step and/or of a later tabletting step, where provided. A suitable processing aid preferably functions as a plasticizer or lubricant. These aids include a solid soap; an acrylic/ maleic anhydride copolymer.

Suitable nonionic surfactants include alkoxylated alcohols, particularly alkoxylated fatty alcohols. These include ethoxylated and propoxylated fatty alcohols, as well as ethoxylated and propoxylated alkyl phenols, both having alkyl groups, suitably linear or secondary, of from 7 to 18, more preferably 8 to 16 carbon chains in length, and an average of 2 to 20 moles, preferably 2 to 10, most preferably 4 to 6 moles of alkylene oxide per mole of alcohol or phenol. Ethoxylated compounds are generally preferred.

Another class of nonionic surfactants that may be used are sorbitan esters of fatty acids, typically fatty acids having from 10 to 24 carbon atoms, for example sorbitan mono oleate.

Other classes of nonionic surfactants that may be used are amine oxides and polyhydroxy fatty acid amides.

Preferably the processing aid, where provided, is present in an amount of from 1-10%, preferably 2-8%, more preferably 3-5% (weight/weight of cleaning agent).

The tower spray powder may include further zeolite, but this is not essential. When there is thus an input of further zeolite, the further zeolite preferably provides 4-30%, more preferably 6-20%, of the cleaning agent (weight/weight). Preferably, when there is a further input of zeolite it is less than the input of zeolite from the zeolite powder added to the tower spray powder.

Suitable inorganic sodium salts may be selected from sodium silicate, sodium carbonate and sodium sulphate. Advantageously each of these salts is present, and each, preferably, is in the range 4-15%, most preferably 5-12% (calculated as anhydrous amount).

Additional constituents of the tower spray powder may be selected from a stabilizer, particularly for a per compound or an enzyme. Suitable stabilizers are salts of polyphosphonic acids, such as 1-hydroxyethane-1,1-diphosphonic acid (HEDP), diethylenetriaminopentamethylene phosphonic acid (DETPMP), ethylenediaminotetramethylene phosphonic acid (EDTMP) and aminotrimethylene phosphonic acid (ATP).

Another useful additional constituent of the cleaning agent is an optical brightener, for example a suitable stilbene compound, in particular diaminostilbene disulfonic acid or a derivative thereof, especially an alkali metal salt. An optical brightener may conveniently be delivered via the tower spray powder.

Another possible additional constituent of the cleaning agent is a soil redeposition inhibitor, for example one or more of polyvinyl pyrollidone, carboxymethyl-cellulose-sodium salt (CMC) or methylcellulose (MC). A soil redeposition inhibitor may conveniently be delivered via the tower spray powder.

Preferably the additional constituents of the tower spray powder do not comprise in total more than 10% of the tower spray powder (weight/weight). Typically each individual additional constituent will not comprise more than 2% of the tower spray powder (weight/weight).

Preferably the flowable zeolitic powder comprises at least 80 wt% zeolite, and preferably at least 90 wt% zeolite.

In this specification references to "zeolite" are to substantially virgin zeolite, including bound water of crystallisation and any atmospherically absorbed unbound water that may be present, but not including deliberately added materials. "Zeolitic powder" denotes zeolite (as just defined) and also such a material containing deliberately added.material(s).

Definitions which refer to the weight or weight ratio of zeolitic powder are made with reference to the zeolite (as defined above) in the zeolitic powder, unless otherwise stated.

It should be noted that both the tower spray powder and the flowable zeolitic powder are preferably macroscopically dry when delivered to the pellet mill. Preferably, both are free-flowing. The amount of liquid components present (if any) must not be such that the respective powders become damp, or sticky, or prone to form lumps. Zeolite for use in the present invention is desirably stored in conditions which discourage water take-up from the atmosphere; for example it can be stored in closed or sealed plastic sacks.

We believe that the invention can be applied using any type of zeolite, including zeolite MAP, zeolite X and zeolite P. Other suitable types are the natural materials analcite, chabazite, heulandite, stilbite, faujasite, natrolite and thomsite. Preferred zeolite for use in the present invention, however, is zeolite A.

The tower spray powder and the zeolitic powder are preferably mixed upstream of the pellet mill in a separate unit, for example a vertical mixer/granulator, a horizontal mixer/granulator or a tumbler unit, all of which are conventional. Preferably, no heating is provided during this step.

Preferably the zeolite content of the pellets is at least 35%, more preferably at least 40%. Most preferably, it is at least 45% and, especially, at least 50%.

Preferably, the zeolite content of the pellets does not exceed 80%, more preferably 70%, most preferably the zeolite content of the pellets does not exceed 65%.

We have found that using the feed materials defined above, pelletisation in a standard pellet mill, e.g. a Kahl mill or a UMT mill, is efficient and unproblematic. This was unexpected given the failure we encountered in trying to extrude such materials.

Further information on pellet mills is readily available. Examples of patents concerning rotary pellet mills include DE 3813081, DE 3806945 and DE 3432780.

Preferably external heat is not provided in the pelletising step. We have found that the temperature of the material being pelletised rises moderately, typically to temperatures in the range 30-55°C, without detriment.

For the pelletisation step, the tower spray powder and the flowable zeolitic powder, as defined above, are preferably mixed together without any further material.

The pellets which are products of the pellet mill are chopped strands, "shaved" from the outer wall of the pellet mill as pelletisation proceeds. Based on our work to date it does not seem necessary from a technical standpoint to treat the pellets in any way before mixing them with post-mixed ingredients, to form the end laundry cleaning agent. However, they could if wished, primarily for aesthetic reasons, be given a simple mechanical treatment in a "ploughshare" shovel mixer, to reduce their mean aspect ratio, to be as close as possible, what may be considered to be the aesthetic ideal, 1:1 (pellet length:maximum diameter). We have found it easy to reduce the mean aspect ratio of the as-formed pellets, by feeding them straight from the pellet mill into the shovel mixer, preferably when the pellets are still warm.

Alternatively or additionally pellets may be spheronized. Preferably, however, the pellets are not spheronized.

Alternatively or additionally pellets may be dusted with a powder to aid flowability. This could suitably be zeolite, for example zeolite A. Preferably, however, the pellets are not dusted.

Suitably the mean aspect ratio of the pellets used in the post-mixing is in the range 0.5-5:1, more preferably 0.8-3:1 (pellet length:maximum diameter). Preferably the pellets are circularly cylindrical and so the aspect ratio denotes length:diameter. Preferably the pellets from the pellet mill are given a mechanical treatment to reduce their mean aspect ratio, to be within this range.

The pellets are intended as a universal base material to which the post-mixing ingredient(s) can be added, for example to make a heavy duty laundry detergent product, or a color care laundry detergent product. Thus, the pellets themselves preferably do not contain any of the "specialist" ingredients which are characteristic of such products. In particular, the pellets preferably do not contain any enzymes, bleaching compounds or bleach activators.

The post-mixing ingredient(s) will depend on the target use for the laundry cleaning agent - for example for general purpose laundry; for heavy duty/white clothes; or for colored clothes. Typically the ratio of the pellets to the post-mixing ingredient(s) is in the range of 20-80 : 80-20 (weight/weight). Preferably the ratio is in the range of 40-70 : 60-30. Most preferably, the ratio is in the range 50-60 : 50-40.

The post-mixing ingredient(s) suitably include one or more of the following: a surfactant, for example an anionic and/or nonionic surfactant; sodium bicarbonate; sodium carbonate; sodium citrate; an anti-foaming agent; an enzyme; a bleaching agent; a bleach activator; a stabilizer, for example of the phosphonate type as defined above; a soil release polymer; a soil redeposition inhibitor; an optical brightener; a fabric softener; a colorant; and a fragrance.

Generally the surfactant component of the post-mixing ingredient(s) is relatively small, suitably making up not more than 10% of the total weight of post-mixing ingredient(s). As mentioned above the post-mixing ingredients may include an alcohol sulphate and this is preferably the only anionic surfactant component, and preferably the only surfactant component, in the post-mixing ingredient(s). In the case of a heavy duty cleaning agent the major complement of post-mixing ingredient(s) is a bleaching agent, for example sodium percarbonate, and a bleach activator, for example TAED; together preferably constituting at least 50% of the weight of post-mixing ingredient(s). In the case of cleaning agents for coloured clothes one or more enzymes, for example, protease, amylase and cellulase, may comprise at least 2% of the weight of post-mixing ingredient(s). At least 40% of the weight of post-mixing ingredient(s) may be made up of sodium bicarbonate and/or sodium carbonate and/or sodium citrate.

A particulate laundry cleaning agent may be made by simple mixing of the pellets and the post-mixing ingredient(s), for example in a tumbler unit. The bulk density of the resulting particulate material is typically high, suitably at least 750g/l, preferably at least 800 g/l. Although such particulate material is itself of potential utility as a washing powder, preferred laundry cleaning agents of the present invention are laundry tablets. Therefore, the invention preferably includes the step, after the step of mixing the pellets with the other ingredients, of pressing the particulate material to form a tablet. As is commonplace the tablet may be formed with two or more layers of different composition, thereby keeping apart any materials which it would be undesirable to mix prior to use - for example a bleach and a bleach activator; or bleach and enzymes.

Pressing the pellets and other ingredients to form tablets is a straightforward step, using standard equipment, for example a commercially available Korsch or Bonals press. It is preferred that when tablets are to be produced, one of the post-mixing ingredient(s) is a disintegrant, for example a rapidly water-swellable material, especially a water-swellable cellulosic material. However, whereas we have previously found it necessary to incorporate at least 10% of a disintegrant in tablets, the tablets made in accordance with the present invention we find that a smaller amount can be employed perfectly adequately. Preferably the disintegrant provides less than 10% of the total weight of the tablets of the present invention and preferably not more than 8%.

We have found that by means of the present invention tablets of very high density may be produced. This is significant because, for a given cleaning power, the tablets are smaller than prior tablets, and this brings about several significant advantages. For example, they may fit in washing machine drawers whereas larger tablets do not.

Preferably the tablets produced in accordance with the present invention have a density of at least 1 kg/l. More preferably, the tablets have a density of at least 1.1 kg/l and most preferably at least 1.15 kg/l.

Preferably the tablets have a hardness of at least 50 N, preferably at least 80 N, as measured by a dynamometer as the maximum force required to break the upper surface of the tablet when a perpendicular force is applied to the centre of it, by a vertically orientated cylinder of diameter 0.5cm.

Preferably the tablets have a disintegration time of not more than 30 seconds, more preferably not more than 25 seconds, most preferably not more than 20 seconds, as measured by a standard method in which a laundry tablet is placed in a stainless steel mesh ladle, with mesh holes approximately 5mm x 5mm, and then successively lowered into and raised from a transparent tank containing 800 ml water at 20°C at a frequency of 60 immersions per minute. When no solid residue of the tablet can be seen within the ladle, the time is recorded ("disintegration time").

Preferably the pellets, and the other ingredients of the washing powder or of the particulate material to be tabletted, are of size such that at least 90 wt% thereof are in the size range 150-1200 µm, more preferably in the size range 250-1000 µm (as determined by standard mesh test, employing ASTM sieves and a Retsch vibrator with predetermined amplitude and working time).

If necessary the pellets and/or the particulate material resulting from the post-mixing may be graded, and overly large or small particles removed, for example for recycling.

When manufactured by the method described herein it will be appreciated that the laundry tablets may have an exceptional combination of beneficial properties, namely high density, high zeolite content and a low amount of disintegrant (all of which would normally lead to long disintegration time); and yet, unexpectedly, exhibit a short disintegration time.

Prior tablets have contained large amounts of silicates as builders. Solid laundry cleaning agents made using the present invention, whether washing powders or laundry tablets, do not require such high amounts of such silicates. Preferably the content of silicon-containing compounds (not including zeolite) in the laundry cleaning agent is less than 10%, more preferably less than 5%.

Preferably the solid laundry cleaning agents contain no phosphate detergents.

Preferably the amount of surfactants in the cleaning agent is at least 10% by weight. Preferably it does not exceed 30%, more preferably 25%, by weight.

In the first aspect of the invention, preferably the zeolite content of the cleaning agent is at least 15% by weight, more preferably at least 20%, most preferably at least 25%, and, especially at least 30%.

A solid laundry cleaning agent may comprise a premix of a flowable tower spray and a flowable zeolitic powder formed into pellets in a pellet mill, the resulting pellets having a zeolite content of at least 30% (weight of zeolite/weight of pellets); and other ingredients mixed with the premix to form the cleaning agent, the zeolite content of the cleaning agent being at least 15% (weight of zeolite/weight of cleaning agent), wherein the zeolitic powder is a zeolite admixed with up to 10% of a processing aid (weight or processing aid/weight of zeolitic powder including processing aid), the processing aid being selected from a nonionic surfactant; an acrylic polymer or copolymer; starch or a derivative thereof; gelatin; polyvinyl alcohol; soap; and water.

The invention will now be further described with reference to the following non-limiting examples.

### Preparation of Tower Spray Powder

A tower spray powder having the following ingredients was prepared in the conventional manner, in a vertical tower, from an aqueous slurry.

| | % |
|---|---|
| 9-13 LAS | 32.0 |
| Sodium tallow soap | 4.0 |
| DTPMP acid | 0.7 |
| Acrylic/maleic acid anhydride copolymer | 5.0 |
| Optical brightener (amino morpholino stilbenic) | 0.69 |
| Zeolite A (MICOLAN 1 - trade mark) | 28.2 |
| CMC | 1.01 |
| Sodium silicate | 7.0 |
| Sodium carbonate | 7.43 |
| Sodium sulphate | 10.54 |
| Water & minors | 3.43 |
| TOTAL | 100.0 |

### Preparation of Pellets A (Reference example)

The tower spray powder was produced in standard manner. The soap was in the form of powder waste from soap production. The tower spray powder was mixed in equal weight with dry, virgin zeolite A powder (MICOLAN 1), in a tumbler mixer. The zeolite had been stored in sealed plastic sacks and nothing was added to it before the mixing. The mixed material was fed into a Kahl pellet mill operated at 100 rpm to yield circularly cylindrical pellets, 1.3mm in diameter and approximately 8-10mm in mean length. The temperature of the pellets as they issued from the pellet mill was about 30-40°C. They were passed directly to a Lödige batch mixer, in which a short treatment with rotating ploughshare shovels reduced the mean length of the pellets to approximately 2-4mm. At this point they were graded using a sieve, to remove powder for recycling.

With the zeolite A also in the tower spray powder, zeolite A made up 64.1% of the weight of Pellets A.

### Production of Pellets B

Production was the same as for Pellets A, but instead of dry, virgin zeolite A being used as the zeolitic powder, zeolitic powder was used, made up of 90% of the dry, virgin zeolite A and 10% soap as described above (weight:weight). This zeolitic powder was mixed in equal weight with the tower spray powder.

Thus, the resultant Pellets B were made up of the following weight proportions:
50:45:5, tower spray ingredients: zeolite A added to the tower spray powder:soap.

With the zeolite A in the tower spray powder, zeolite A made up 59.1% of the weight of Pellets B.

### Production of High Density Washing Powder for Coloreds (Reference example)

Pellets A as described above were post-mixed with the following ingredients in a standard tumbler mixer in the proportions stated to yield a high density washing powder intended for washing colored fabrics.

| Ingredients | % |
|---|---|
| Pellets A | 60.00 |
| Fatty alcohol sulphate needles | 4.5 |
| C₁₃₋₁₅ Aliphatic alcohol, ethoxylated (7 EO) | 5.0 |
| Sodium carbonate | 12.97 |
| Sodium citrate dihydrate | 10.0 |
| Antifoam powder (polysiloxane supported on starch) | 1.93 |
| Enzymes (protease, amylase, cellulase) | 2.8 |
| Soil release polymer (polyethylene glycol/polyester compound) | 1.5 |
| HEDP | 0.8 |
| Perfume | 0.5 |
| TOTAL | 100.00 |

### Preparation of Laundry Tablet for Coloreds

The ingredients set out in the table below were mixed together in a standard tumbler mixer, fed repetitively to a Korsch tablet press, and pressed into white monolayer tablets of circularly cylindrical shape, having the following characteristics:
Size - 22mm height x 44mm diameter
Density - 1.17 kg/l
Hardness - 90N (measured as described above)
Disintegration time - 20 seconds (measured as described above)
Weight: 37.5g

| Ingredients | % |
|---|---|
| Pellets B | 55.0 |
| Fatty alcohol sulphate needles | 4.35 |
| Sodium carbonate | 16.29 |
| Sodium citrate dihydrate | 10.41 |
| Antifoam powder (polysiloxane supported on starch) | 1.93 |
| Enzymes (protease, amylase, cellulase) | 2.63 |
| Soil release polymer (polyethylene glycol/polyester compound) | 1.0 |
| HEDP | 0.69 |
| Granular cellulose disintegrant | 7.50 |
| Perfume | 0.20 |
| TOTAL | 100.0 |

### Production of Laundry Tablets for Heavy Duty/Whites

This tablet was composed of two layers, produced in standard manner in a Korsch press. The two layers are made up as follows.

| | Blue Phase | White Phase | Finished tablet (30% blue + 70% white) |
|---|---|---|---|
| Pellets B | 55.0 | 55.0 | 55.0 |
| Fatty alcohol sulphate needles | 4.00 | 4.00 | 4.00 |
| Nonionic surfactant (C₁₃₋₁₅ alkyl, 5 EO) | 3.5 | 1.00 | 1.75 |
| Silicate builder | 9.64 | 1.53 | 3.96 |
| Sodium percarbonate | - | 28.57 | 20.00 |
| Bleach activator (TAED) | 15.0 | - | 4.50 |
| Enzymes (protease, amylase, cellulase) | 2.66 | - | 0.80 |
| Granular disintegrant | 7.00 | 7.00 | 7.00 |
| Antifoam (as above) | 0.27 | 0.27 | 0.27 |
| Blue dye | 0.013 | - | 0.004 |
| Perfume | - | 0.29 | 0.2 |
| Water & minors | to 100.00 | to 100.00 | to 100.00 |

| | | | |
|---|---|---|---|
| (weight percentages stated) | | | |

The silicate builder had a ratio of SiO₂:Na₂O of 2.85:1 (weight:weight). The resulting two layer disc-shaped tablet had the following characteristics.
Size - 22mm height × 44mm diameter
Density - 1.15 kg/l
Hardness - 100N (measured as described above)
Disintegration time - 15 seconds (measured as described above)
Weight: 37.5g

### Production of Washing Powder for Heavy Duty/Whites

Pellets B as described above were mixed together with further ingredients in a standard tumbler mixer in the proportions stated below to yield a high density washing powder intended for washing heavily soiled white fabrics.

| Pellets B | 60.0 |
|---|---|
| Alcohol sulphate granules | 4.32 |
| Nonionic surfactant (C₁₃₋₁₅ alkyl, 5 EO) | 3.00 |
| Silicate builder | 4.00 |
| Sodium percarbonate | 20.00 |
| Bleach activator (TAED) | 4.50 |
| Enzymes (protease, amylase) | 0.80 |
| Antifoam powder 4256 | 0.27 |
| Perfume | 0.5 |
| Water & minors | to 100.00 |

| | |
|---|---|
| (weight percentages stated) | |

## Claims

1. A method of making a solid laundry cleaning agent, comprising the steps of pelletising a flowable tower spray powder and a flowable zeolitic powder in a pellet mill to form a premix comprising pellets with a zeolite content of at least 30% (weight of zeolite/weight of pellets); and mixing the pellets with the other ingredient(s) of the solid laundry cleaning agent, wherein the zeolitic powder is a zeolite admixed with up to 10% of a processing aid (weight of processing aid/weight of zeolitic powder including processing aid), the processing aid being selected from a nonionic surfactant; an acrylic polymer or copolymer; starch or a derivative thereof; gelatin; polyvinyl alcohol; soap; and water.

2. A method as claimed in claim 1 wherein the pellets have a zeolite content of at least 40%.

3. A method as claimed in claim 1 or 2 wherein the zeolitic content of the pellets does not exceed 80%.

4. A method as claimed in claim 1,2 or 3, wherein the processing aid is in solid form.

5. A method as claimed in claim 4, wherein the processing aid is a sodium and/or potassium soap of a fatty acid selected from a tallow fatty acid, coconut oil fatty acid, palm kernel oil fatty acid, oleic acid and stearic acid, the soap being in particulate form.

6. A method as claimed in any preceding claim wherein said zeolitic powder comprises zeolite A.

7. A method as claimed in any preceding claim wherein the tower spray product is made up of the following constituents (weight of constituents/weight of tower spray powder):
20-60% anionic surfactant(s)
0-15% processing aid(s)
0-25% further zeolite(s)
12-45% inorganic alkali metal salts(s)
0-20% additional constituent(s)

8. A method as claimed in any preceding claim comprising the step, after pelletisation, of mechanically treating the pellets to reduce their aspect ratio.

9. A method as claimed in any preceding claim wherein the ratio of pellets to said other ingredient(s) is in then range 20-80: 80-20 (weight of pellets/weight of said other ingredients).

10. A method as claimed in claim 9 wherein the ratio of pellets to said other ingredient(s) is in the range 40-70: 60-30.

11. A method as claimed in any preceding claim wherein said other ingredient(s) include one or more of the following:
a surfactant; sodium bicarbonate; sodium carbonate; sodium citrate; an antifoaming agent; an enzyme; a bleaching agent; a bleach activator; a stabilizer; a soil release polymer; a soil redeposition inhibitor; a fabric softener; a colorant; and a fragrance.

12. A method as claimed in any preceding claim wherein the resulting particulate material has a bulk density of at least 750 g/l.

13. A method as claimed in any preceding claim comprising the step, after said mixing step, of pressing the particulate material to form a tablet.

14. A method as claimed in claim 13 wherein said other ingredient(s) include a disintegrant.

15. A method as claim in claim 13 or 14 wherein the tablet has a density of at least 1 kg/l.

16. A method as claimed in claim 13 wherein the tablet has a density of at least 1.1 kg/l.

## Patentansprüche

1. Verfahren zur Herstellung eines festen Waschmittels, umfassend die Schritte, ein fließfähiges Turmsprühpulver und ein fließfähiges zeolithisches Pulver in einer Pelletieranlage zu pelletieren, um ein Vorgemisch zu bilden, das Pellets mit einem Zeolithgehalt von wenigstens 30% (Gewicht des Zeoliths / Gewicht der Pellets) umfasst; und die Pellets mit dem bzw. den anderen Inhaltsstoff(en) des festen Waschmittels zu vermischen, wobei das zeolithische Pulver ein Zeolith ist, dem bis zu 10% eines Verarbeitungshilfsstoffes (Gewicht des Verarbeitungshilfsstoffes / Gewicht des zeolithischen Pulvers einschließlich Verarbeitungshilfsstoff) beigemischt sind, wobei der Verarbeitungshilfsstoff aus einem nichtionischen Tensid, einem Acrylpolymer oder -copolymer, Stärke oder einem Derivat daraus, Gelatine, Polyvinylalkohol, Seife und Wasser ausgewählt ist.

2. Verfahren gemäß Anspruch 1, wobei die Pellets einen Zeolithgehalt von wenigstens 40% haben.

3. Verfahren gemäß Anspruch 1 oder 2, wobei der Zeolithgehalt der Pellets 80% nicht überschreitet.

4. Verfahren gemäß Anspruch 1, 2 oder 3, wobei der Verarbeitungshilfsstoff Festform hat.

5. Verfahren gemäß Anspruch 4, wobei der Verarbeitungshilfsstoff eine Natrium- und/oder Kaliumseife aus einer Fettsäure ist, die aus einer Talgfettsäure, Kokosölfettsäure, Palmkernölfettsäure, Oleinsäure und Stearinsäure ausgewählt ist, wobei die Seife partikuläre Form hat.

6. Verfahren gemäß einem der vorhergehenden Ansprüche, wobei das zeolithische Pulver Zeolith A umfasst.

7. Verfahren gemäß einem der vorhergehenden Ansprüche, wobei das Turmsprühprodukt aus den folgenden Bestandteilen besteht (Gewicht der Bestandteile / Gewicht des Turmsprühpulvers):
20 - 60% anionische(s) Tensid(e)
0 - 15% Verarbeitungshilfsstoff(e)
0 - 25% weitere(s) Zeolith(e)
12 - 45% anorganische(s) Alkalimetallsalz(e)
0 - 20% zusätzliche(r) Bestandteil(e)

8. Verfahren gemäß einem der vorhergehenden Ansprüche, nach der Pelletierung den Schritt umfassend, die Pellets mechanisch zu bearbeiten, um ihr Aspektverhältnis zu reduzieren.

9. Verfahren gemäß einem der vorhergehenden Ansprüche, wobei das Verhältnis der Pellets zu dem bzw. den anderen Inhaltsstoff(en) im Bereich von 20 - 80 : 80 - 20 liegt (Gewicht der Pellets / Gewicht der anderen Inhaltsstoffe).

10. Verfahren gemäß Anspruch 9, wobei das Verhältnis der Pellets zu dem bzw. den anderen Inhaltsstoff(en) im Bereich von 40 - 70 : 60 - 30 liegt.

11. Verfahren gemäß einem der vorhergehenden Ansprüche, wobei der bzw. die andere(n) Inhaltsstoff(e) einen oder mehrere der folgenden Inhaltsstoffe aufweisen:
ein Tensid; Natriumbicarbonat; Natriumcarbonat; Natriumcitrat, ein Antischaummittel; ein Enzym; ein Bleichmittel; einen Bleichaktivator; einen Stabilisator; ein Schmutzlösepolymer; einen Vergrauungsinhibitor; einen Textilweichmacher; einen Farbstoff und einen Duftstoff.

12. Verfahren gemäß einem der vorhergehenden Ansprüche, wobei das entstehende partikuläre Material eine Schüttdichte von wenigstens 750 g/l hat.

13. Verfahren gemäß einem der vorhergehenden Ansprüche, nach dem Schritt des Mischens den Schritt umfassend, das partikuläre Material zu pressen, um eine Tablette auszubilden.

14. Verfahren gemäß Anspruch 13, wobei der bzw. die andere(n) Inhaltsstoff(e) ein Abbaumittel aufweisen.

15. Verfahren gemäß Anspruch 13 oder 14, wobei die Tablette eine Dichte von wenigstens 1 kg/l hat.

16. Verfahren gemäß Anspruch 13, wobei die Tablette eine Dichte von wenigstens 1,1 kg/l hat.

## Revendications

1. Un procédé pour faire un produit de nettoyage de linge solide, comprenant les étapes de pastillage d'une poudre de bec de pulvérisation pouvant ruisseler et d'une poudre de zéolite pouvant ruisseler dans une presse de pastillage pour former un prémélange comprenant des pastilles avec une teneur en zéolite d'au moins 30% (poids de zéolite/poids des pastilles) ; et de mélange des pastilles avec l'autre ingrédient(s) du produit de nettoyage de linge solide, où la poudre de zéolite est un zéolite mélangé avec jusqu'à 10% d'adjuvant de fabrication (poids d'adjuvant de fabrication/poids de poudre de zéolite incluant l'adjuvant de fabrication), l'adjuvant de fabrication étant sélectionné parmi un surfactant non ionique, un polymère acrylique ou copolymère, l'amidon ou un dérivé de celui-ci, la gélatine, l'alcool polyvinylique, le savon, et l'eau.

2. Un procédé comme revendiqué en revendication 1 où les pastilles ont une teneur en zéolite d'au moins 40%.

3. Un procédé comme revendiqué en revendication 1 ou 2, où la teneur en zéolite des pastilles n'excèdent pas 80%.

4. Un procédé comme revendiqué en revendication 1, 2 ou 3 où l'adjuvant de fabrication est dans une forme solide.

5. Un procédé comme revendiqué en revendication 4, où l'adjuvant de fabrication est un savon de soude et/ou de potassium d'un acide gras sélectionné parmi un acide gras de suif, un acide gras d'huile de noix de coco, un acide gras d'huile de palmite, un acide oléique et un acide stéarique, le savon étant en forme particulaire.

6. Un procédé comme revendiqué dans l'une des revendications précédentes où une poudre de zéolite comprend le zéolite A.

7. Un procédé comme revendiqué dans l'une des revendications précédentes où le produit du bec de pulvérisation est fait à partir des constituants suivants (poids des constituants/poids de la poudre du bec de pulvérisation) :
20-60% surfactant(s) anionique(s)
0-15% adjuvant(s) de fabrication
0-25% autre(s) zéolite(s)
12-45% sel(s) de métal alcalin inorganique(s)
0-20% constituant(s) additionnel(s)

8. Un procédé comme revendiqué dans l'une des revendications précédentes comprenant l'étape, après pastillage, de traitement mécanique des pastilles pour réduire leur rapport de longueurs.

9. Un procédé comme revendiqué dans l'une des revendications précédentes où le ratio des pastilles par rapport au(x)dit(s) autre(s) ingrédient(s) est dans la fourchette de 20-80 : 80-20 (poids de pastilles/poids desdits autres ingrédients).

10. Un procédé comme revendiqué dans la revendication 9 où le ratio des pastilles par rapport au(x)dit(s) autre(s) ingrédient(s) est dans la fourchette de 40-70 : 60-30.

11. Un procédé comme revendiqué dans l'une des revendications précédentes où le(s)dit(s) autre(s) ingrédient(s) incluent un ou plusieurs parmi les suivants :
un surfactant ; bicarbonate de sodium ; carbonate de sodium ; citrate de sodium ; un agent antimoussant ; une enzyme ; un agent de blanchiment ; un activateur de blanchiment ; un stabilisateur ; un polymère antisalissure ; un inhibiteur de dépôt de salissure ; un produit assouplissant ; un colorant ; et un parfum.

12. Un procédé comme revendiqué dans l'une des revendications précédentes où le matériau particulaire résultant a une densité apparente d'au moins 750 g/l.

13. Un procédé comme revendiqué dans l'une des revendications précédentes comprenant l'étape après ladite étape de mélange, de presser le matériau particulaire pour former un comprimé.

14. Un procédé comme revendiqué dans la revendication 13 où le(s)dit(s) autre(s) ingrédient(s) incluent un délitant.

15. Un procédé comme revendiqué dans la revendication 13 ou 14 où le comprimé a une densité d'au moins 1 kg/l.

16. Un procédé comme revendiqué dans la revendication 13 où le comprimé a une densité d'au moins 1,1 kg/l.
